

## UNITED STATES PATENT OFFICE

2,394,978

## REFINING PROCESS

Richard C. Brandon, Elizabeth, N. J., assignor to  
Standard Oil Development Company, a corpora-  
tion of Delaware

No Drawing. Original application April 2, 1942,  
Serial No. 437,364. Divided and this applica-  
tion December 12, 1942, Serial No. 468,814

7 Claims. (Cl. 260—627)

The present application is a division of my co-  
pending application Serial No. 437,364, filed April  
2, 1942.

The present invention relates to improvements  
in the refining of hydrocarbon oils and, more par-  
ticularly, it relates to an improved method for  
inhibiting petroleum distillates, such as gasoline,  
to produce a refined product which is stable  
against gum formation.

It is generally known that gasoline and other  
hydrocarbon distillates, particularly if they result  
from a cracking operation, contain substantial  
quantities of materials which, upon storage, form  
gums. In certain cases, the formation of gum is  
so great that the gasoline or other distillate must  
be redistilled; that is to say, when a hydrocarbon  
oil such as gasoline is treated under certain re-  
fining conditions and shipped to some distant  
bulk station where it remains in storage for weeks  
or even months, there is imminent danger that  
during storage the formation of gummy con-  
stituents in the gasoline and other distillate will  
take place. Obviously the presence of these gum  
constituents in a gasoline is highly undesirable,  
for their presence in the carburetor of an auto-  
mobile seriously interferes with the efficient oper-  
ation thereof.

Prior to my invention, others have proposed the  
addition of so-called gum inhibitors to gasoline  
in order to prevent the formation of the afore-  
mentioned gummy constituents. Among the  
common inhibitors that have been proposed are  
the tricresols (meta, para and ortho cresols) and  
other phenols. While these products are satis-  
factory gum inhibitors, relatively large quanti-  
ties are required, and like many of the other  
commercial gum inhibitors they are also rela-  
tively expensive.

It is the main purpose of my present inven-  
tion to provide means for producing a gum in-  
hibitor which is satisfactory from the stand-  
point of effectiveness and whose use affords substantial  
economies.

Briefly, my present process involves treating a  
gasoline to prevent gum formation with cata-  
lytically cracked petroleum alkylated phenols.

Other objects of my invention will appear from  
the following more detailed description and  
claims.

In order to illustrate my invention more fully,  
the following specific example is set forth with  
the understanding that the precise details enum-  
erated herein are purely illustrative and do not  
impose any limitation thereon.

## Example

A West Texas gas oil was extracted with 1%  
by volume of a 40% aqueous sodium hydroxide  
solution. The treatment with caustic soda re-  
sulted in the formation of a three-liquid phase  
system. The system consisted of an upper oil  
layer, an intermediate sodium phenolate layer,  
and a lower caustic soda solution layer. The  
several layers were separated by decantation,  
whereupon the intermediate phenolate layer was  
treated with  $\text{CO}_2$  although other acidic material  
could have been used in order to convert the  
phenolates into the corresponding phenols. The  
exact amount of acidic material necessary to  
effect the desired conversion will of course de-  
pend on the quantity of phenolate present. How-  
ever, care must be taken in precipitating the  
phenols, since the caustic soda extract also con-  
tains naphthenic acids so that an acidic mate-  
rial must be employed which will cause the afore-  
mentioned fractional precipitation or selective  
precipitation of the desired phenols. The acidified  
precipitate was freed of asphaltic material  
by vacuum distillation during which 70% of the  
material was taken overhead as a product, the  
bottoms being discarded. The distillate thus ob-  
tained contained alkylated phenols.

The distillate obtained as hereinbefore ex-  
plained was then catalytically cracked in the  
presence of a cracking catalyst consisting of acid  
treated Montmorillonite clay. However, a syn-  
thetic gel catalyst, say one consisting of silica  
and alumina gels could have been used. During  
the cracking operation, the distillate was vapor-  
ized and then heated to a temperature of 830° F.,  
whereupon it was contacted with the aforesaid  
catalyst. The reaction products were then con-  
densed and fractionated and a fraction boiling  
within the range of from about 120—402° F. at  
25 mm. pressure was recovered. The yield of this  
product was approximately 75% on feed.

When 10 mg. of this material was added to 100  
ml. of gasoline, the "breakdown time" was 270  
minutes.

It should be explained that the "breakdown"  
time is a commonly used method for determin-  
ing in the laboratory the effectiveness of an addi-  
tion agent as a gum inhibitor. The determina-  
tion is made by introducing 25 cc. of the gasoline  
into a test tube which is then inserted into a  
bomb. The bomb is placed under 100 lbs. oxygen  
pressure at room temperature and then heated to  
a temperature of 212° F. The time elapsed be-  
fore there is a 2 lbs. drop in pressure as measured

from the maximum pressure attained in the bomb is recorded as the breakdown period.

It should be noted that in the text hereinbefore mentioned, the base gasoline (the gasoline containing no inhibitor) had a breakdown itself of 100 minutes and therefore the inclusion of 10 mg. of the catalytically cracked phenols increased the resistance to gum formation by an amount equal to 170%.

In order to show the utility of my present invention, I submit the following data. In making the below comparative tests, tricresol was used on the one hand and the product of Example 1 on the other hand, in the manner indicated in the said table:

|                     | Tricresol       |     | Cracked alkylated phenols |
|---------------------|-----------------|-----|---------------------------|
| Amount added.....   | milligrams..... | 10  | 10                        |
| Breakdown time..... | minutes.....    | 170 | 290                       |

It will be noted from the above data in which a standard commercial gasoline was treated with both the tricresol and the cracked alkylated phenols that the cracked alkylated phenols were approximately twice as effective as the commercial tricresol inhibitor.

Also, it should be pointed out that the phenols before cracking had a sulfur content of 0.6%, while after cracking this quantity was reduced to 0.28% which means of course that the cracked phenols introduced less sulfur into the treated gasoline. With respect to color, it is pointed out that the alkylated phenols before cracking had a color of 1 Robinson, whereas after cracking the phenols had a color of 18 Robinson.

In a further test where 20 mg. of the uncracked alkylated phenols were added to another portion of the above mentioned standard commercial gasoline, the breakdown time was 310 minutes. It is obvious from the above data therefore that one part of the cracked alkylated phenols has approximately the same effect in inhibiting gum formation as do two parts of the uncracked alkylated petroleum phenols.

In the cracking of the petroleum phenol hereinbefore described in the specific example, it should be pointed out that the conditions therein set forth, while preferred are not the only conditions under which good results may be obtained. For instance, the cracking temperature may vary from 800-1000° F. The phenols may be fed in a continuous operation to the cracking zone at a flow rate of from 0.2-2.0 volumes of phenol per volume of reaction zone per hour, and the pressures may vary from subatmospheric pressure to atmospheric pressure, or thereabouts.

Instead of using  $\text{CO}_2$ , I may use a strongly acidic material such as the mineral acids, but the quantity added must be carefully controlled to precipitate only phenols and leave naphthenates and other undesired constituents in solution in known manner.

To recapitulate, my invention resides in the concept of catalytically cracking alkylated phenols of petroleum origin and employing the reaction products as addition agent to hydrocarbon oils such as gasoline, where they serve as inhibitors. Since these products have a very high degree of effectiveness, smaller quantities may be used, and therefore their use affords a substantial economy.

10 Many modifications of my invention falling within the spirit thereof will readily suggest themselves to those familiar with this art, and it is my intention to claim all of the subject matter herein disclosed and all modifications which 15 are included by necessary implication except that subject matter excluded by the terms of the appended claims.

What I claim is:

1. The method of preparing cracked phenols 20 which comprises subjecting a petroleum fraction to the action of caustic soda, separating an extract phase containing alkylated phenols, treating said extract with a precipitant for phenols selected from the group consisting of carbon dioxide and mineral acids so as to precipitate the phenols while leaving naphthenates in solution and subjecting the precipitated phenols to catalytic cracking at a temperature of the order of 800° to 1,000° F., a pressure not substantially 25 above atmospheric and a flow rate of the order of 0.2 to 2.0 volumes of phenol per volume of reaction zone per hour, in the presence of an acid treated clay catalyst.

2. The method of claim 1 wherein said petroleum fraction is a gas oil.

3. The method of producing gum inhibitors for stabilizing gasoline which comprises subjecting alkylated phenols derived and separated from petroleum oil to catalytic cracking at a temperature of the order of 800° to 1,000° F., a pressure not substantially above atmospheric and a flow rate of the order of 0.2 to 2.0 volumes of phenol per volume of reaction zone per hour.

4. The method specified in claim 3 wherein the catalyst employed for cracking is an acid treated clay.

5. The method of producing compounds effective to prevent gum formation which comprises subjecting alkylated phenols derived and separated from petroleum hydrocarbons to cracking in the presence of an acid treated clay catalyst.

6. In the method of producing gum inhibitors for gasoline by extracting alkylated phenols from petroleum oil with caustic alkali and precipitating the alkylated phenols with an acid precipitant the improvement which comprises subjecting the precipitated alkylated phenols to catalytic cracking at a temperature of the order of 800° to 1,000° F., a pressure not substantially above atmospheric and a flow rate of the order of 0.2 to 2.0 volumes of phenol per volume of reaction zone per hour.

7. The method set forth in claim 6 wherein an acid treated clay is used as the catalyst.

RICHARD C. BRANDON.